

# United States Patent [19]

Mikami et al.

[11] Patent Number: 4,465,756

[45] Date of Patent: Aug. 14, 1984

[54] ELECTROSTATOGRAPHIC  
ENCAPSULATED TONER MATERIAL  
IMPROVED IN CHARGEABILITY

[75] Inventors: Takeshi Mikami; Noriyuki Hosoi,  
both of Fujinomiya, Japan

[73] Assignee: Fuji Photo Film Co., Ltd., Kanagawa,  
Japan

[21] Appl. No.: 432,064

[22] Filed: Sep. 30, 1982

## [30] Foreign Application Priority Data

Oct. 22, 1981 [JP] Japan ..... 56-169033

[51] Int. Cl.<sup>3</sup> ..... G03G 9/16

[52] U.S. Cl. ..... 430/138; 430/98;  
430/110

[58] Field of Search ..... 730/109, 110, 138

## [56] References Cited

### U.S. PATENT DOCUMENTS

3,431,412 3/1969 Okubo ..... 430/110  
4,259,428 3/1981 Tsuneda ..... 430/138

## OTHER PUBLICATIONS

Sisley Encyclopedia of Surface Active Agents, Chemical Pub. Co., 1952, p. 66.

Primary Examiner—John E. Kittle

Assistant Examiner—John L. Goodrow

Attorney, Agent, or Firm—Toren, McGeady and Stanger

[57]

## ABSTRACT

An electrostatographic toner material suitably employable for the pressure fixing process, which comprises encapsulated toner particles having an average particle size in the range from about 0.5 to 1,000 microns, in which the toner particle comprises a pressure fixable adhesive core material containing a colorant and a pressure rupturable shell enclosing the core material, the outer surface of the shell being provided with a surface active agent having the following hydrophobic group:



in which R<sup>1</sup> and R<sup>2</sup> are the same or different, and each is an aliphatic hydrocarbon group of 2-20 carbon atoms or an aromatic hydrocarbon group of 6-20 carbon atoms.

11 Claims, No Drawings

**ELECTROSTATOGRAPHIC ENCAPSULATED  
TONER MATERIAL IMPROVED IN  
CHARGEABILITY**

This invention relates to an electrostatographic toner material, and more particularly relates to a pressure fixable electrostatographic toner material comprising encapsulated toner particles.

There is known the electrostatography which comprises developing a tone electrostatic latent image contained on a photoconductive or dielectric surface with a toner material containing colorant and a fixing aid to produce a visible toner image, and transferring and fixing the visible toner image onto a surface of a support medium such as a sheet of paper.

The development of the latent image to produce a visible toner image is carried out by the use of either a developing agent consisting of a combination of toner material with carrier particles, or a developing agent consisting of toner material only. The developing process utilizing the combination of toner material with carrier particles is named "two component developing process", while the developing process utilizing only the toner material is named "one component developing process".

The toner image formed on the latent image is then transferred onto a surface of a support medium and fixed thereto. The process for fixing the toner image to the support medium can be done through one of three fixing processes, that is, a heat fixing process (fusion process), a solvent fixing process and a pressure fixing process.

The pressure fixing process which involves fixing the toner material onto the surface of a support medium under application of pressure thereto is described, for instance, in U.S. Pat. No. 3,269,626. The pressure fixing process involving the use of neither the heating procedure nor the solvent produces no such troubles as inherently attached to either the heat fixing process or the solvent fixing process. Moreover, the pressure fixing process can be employed with a high speed automatic copying and duplicating process, and the access time is very short in the pressure fixing process. Accordingly, the pressure fixing process is said to be an advantageous fixing process inherently having a variety of preferable features.

However, the pressure fixing process also has a variety of inadvantageous features. For instance, the pressure fixing process generally provides poorer fixability than the heat fixing process does, whereby the toner image fixed onto a paper is apt to rub off easily. Further, the pressure fixing process requires very high pressure for the fixing, and such a high pressure tends to break the cellulose fibers of the support medium such as paper and also produces glossy surface on the support medium. Moreover, the pressing roller requires to have relatively greater size, because the roller necessarily imparts very high pressure to the toner image on the support medium. Accordingly, reduction of the size of a copying and duplicating machine cannot exceed a certain limit defined by the size of the pressing roller.

There has been previously proposed an encapsulated toner material which comprises toner particles enclosed with micro-capsules, so as to overcome the above-described disadvantageous features of the pressure fixing process. The encapsulated toner material is prepared by enclosing core particles (containing colorant

such as carbon black) with shells which are rupturable by the application of pressure. The so-prepared encapsulated toner material has various advantageous features; for instance, the fixing of the encapsulated toner

5 material does not require very high pressure, and the fixability is excellent. Accordingly, the encapsulated toner material is viewed as suitable for the use in the pressure fixing process. However, the encapsulated toner materials proposed up to now appear unsatisfactory in practical use, because they are not able to satisfy all of the characteristics required for providing smooth copying and duplicating operation and for accomplishing excellent toner image fixability and quality.

More in detail, it is required for the toner material for 10 the use as a dry type developing agent in the electrostatography to have excellent powder characteristics (or, powder flow properties) to provide high development quality, and to be free from staining the surface of the photosensitive material on which the latent image is formed. The term "powder characteristics" particularly means resistance to agglomeration and blocking of the toner particles. In the process for the preparation of an encapsulated toner material, the toner material is generally separated from a toner dispersed solution and dried through a spray-drying procedure. The previously known encapsulated toner material is apt to undergo agglomeration either in the spray-drying process, or in the storage period after the spray-drying. The so-agglomerated toner material markedly degrades the resolution of the visible toner image produced on the electrostatographic latent image, whereby markedly decreasing the sharpness of the visible toner image fixed onto the support medium.

Further, a toner material employed for the two component developing process is also required not to stain the surfaces of the carrier particles. The toner material for the use as a developing agent in the pressure fixing process is furthermore required to be satisfactory in the fixability under pressure and not to undergo off-setting against the roller surface, that is, phenomenon in which the toner adheres to the roller surface so as to stain it.

The encapsulated toner materials proposed until now are not satisfactory, at least, in one of these requirements for the developing agent to be employed for the pressure fixing process.

Moreover, the heretofore proposed encapsulated toner materials can hardly be charged with electron 45 enough for producing a clear toner image on a latent image formed on a photosensitive material. Thus, these toner materials are considered to be unsatisfactory in the developing characteristics. This problem particularly occurs when the two component developing process is employed. In the two component developing process, the encapsulated toner material is given an electric charge opposite to the charge of the electrostatic latent image formed on the photosensitive material, by rubbing the toner material with a carrier such as iron powder or glass beads. The heretofore proposed encapsulated toner materials, however, can hardly be imparted enough electric charge in this process, probably because the shell materials of these toner materials have electric-chargeability relatively close to these of the carriers such as iron powder and glass beads. The chargeability of the shell material can be put apart from that of the carrier by coating the shell with a pertinent polymer material so as to render the toner material more chargeable in the two component developing process. However, the polymer material coated over

the shell is apt to be cracked or separated from the shell under mechanical forces such as friction for a long period, collision, thermal strain and the like in the developing stage.

It is, accordingly, an object of the invention to provide an electrostatographic toner material free from the drawbacks described above.

It is another object of the invention to provide an encapsulated toner material suitable employed for the pressure fixing process and free from the drawbacks described above.

It is a further object of the invention to provide an encapsulated toner material suitable employed for the pressure fixing process, whose powder characteristics are remarkably improved.

It is a still further object of the invention to provide an encapsulated toner material having improved pressure fixability in addition to the improved powder characteristics.

It is a still further object of the invention to provide an encapsulated toner material having improved resistance to the off-setting in addition to the improved powder characteristics and the improved pressure fixability.

It is a still further object of the invention to provide an encapsulated toner material which is resistant to rupture prior to the pressing operation in the pressure fixing process, while which is readily rupturable in the pressure fixing operation.

It is a still further object of the invention to provide an encapsulated toner material which is easily chargeable for producing a visual toner image on a latent image formed on a photosensitive material.

The above-described objects and other objects which will be apparent from the hereinafter-given description are accomplished by the present invention, that is, an electrostatographic toner material comprising encapsulated toner particles having an average particle size in the range from about 0.5 to about 1,000 microns, in which the toner particle comprises a pressure fixable adhesive core material containing a colorant and a pressure rupturable shell enclosing the core material, the outer surface of the shell being provided with a surface active agent having the following hydrophobic group (I):



in which  $R^1$  and  $R^2$  are the same or different, and each is an aliphatic hydrocarbon group of 2-20 carbon atoms or an aromatic hydrocarbon group of 6-20 carbon atoms.

Each of  $R^1$  and  $R^2$  preferably is an aliphatic hydrocarbon group of 4-12 carbon atoms or an aromatic hydrocarbon group of 6-12 carbon atoms, and more preferably is an aliphatic hydrocarbon group of 6-10 carbon atoms.

The surface active agent having the hydrophobic group (I) preferably contains at least one hydrophilic group selected from the group consisting of sulfonate, carboxylate, phosphate, amine, quaternary ammonium salt and pyridinium salt. Most preferred is the sulfonate group.

Representative examples of the surface active agents employable in the invention include:

bis(tridecyl) sodium sulfosuccinate,

dihexyl sodium sulfosuccinate, diisodecyl diethanolamine sulfosuccinate, dibenzyl sodium sulfosuccinate, butyldecyld potassium sulfosuccinate, dipentyl sodium sulfosuccinate, dioctyl sodium sulfosuccinate, di-2-ethylhexyl sodium sulfosuccinate, diisooctyl sodium sulfosuccinate, and phenetyl octyl sodium sulfosuccinate.

The surface active agent having the hydrophobic group can be provided in the form of a solution onto an outer surface of shell of an encapsulated toner material. Such a solution prepared by mixing or dissolving the surface active agent in water, an organic solvent, an aqueous organic solvent or others. The surface active agent-containing solution can be brought into contact with the encapsulated toner in any of the steps for the preparation of the desired toner materials. Preferred is a procedure involving addition of the surface active agent-containing solution to an encapsulated toner-containing dispersion just prior to subjecting it to a drying operation such as one employing a spray dryer. The surface active agent is provided onto the surface of the encapsulated toner material in the amount of 0.0001-10% by weight of the toner material, preferably in the amount of 0.01-1% by weight.

There is no specific limitation on the material of shell of the encapsulated toner according to the invention, as far as the material is pertinent to the production of the shell. Examples of the shell materials include gum arabic, gelatin, polyester, polyamide, polystyrene, polycarbonate, polyether, polyethylene, polyurea, polyurethane, polythiourethane, polythiourea, and copolymers such as poly(styrene-methacrylate) and poly(styrene-acrylate). Preferred are polyurethane, polyurea and polythiourethane.

The shell can be composed substantially of a two or more layers. For instance, the shell can be composed substantially of a double layer comprising a polyurethane, polyurea and/or polythiourethane layer and a polyamide layer.

In the present invention, the term "polyurethane, polyurea and polythiourethane" means a polymer produced by the polycondensation reaction between polyisocyanate and/or polythioisocyanate and one or more of the counterpart compounds such as polyol, polythiol, water, polyamine and piperazine. Accordingly, the term "polyurethane" means either a simple polyurethane comprising substantially the urethane bondings only or a polymer comprising the urethane bondings and a relatively small number of the urea and/or thiourethane bondings. The term "polyurea" means either a simple polyurea comprising substantially the urea bondings only or a polymer comprising the urea bondings and a relatively small number of the urethane and/or thiourethane bondings. In the same way, the term "polythiourethane" means either a simple polythiourethane comprising substantially the thiourethane bondings only or a polymer comprising the thiourethane bondings and a relatively small number of the urethane and/or urea bondings.

The material preferably employed for preparing the shell in the invention is a polycondensation product of polyisocyanate, polyol and water, or a polycondensation product of polyisocyanate, polyol and polyamine.

The electrostatographic toner material of the invention is preferably prepared by a process which comprises encapsulating very small droplets of the pressure

fixable adhesive core material containing a colorant dispersed in an aqueous medium with the pressure rupturable shell material to prepare encapsulated particles; providing the surfaces of the encapsulated particles with the surface active agent; and separating the encapsulated particles from the aqueous medium to obtain dry encapsulated toner materials.

The encapsulation of the droplets of the core material with the shell material can be done by any known method for preparing the so-called micro-capsule containing a hydrophobic liquid, such as the phase separation method as described in U.S. Pat. Nos. 2,800,457 and 2,800,458; the interfacial polymerization as described in Japanese Patent Publications No. 38(1963)-19,574, No. 42(1967)-446 and No. 42(1967)-771, British Patent Nos. 989,264, 950,443, 867,797, 1,069,140 and 1,046,409; the method involving polymerization of a monomer in oil droplets as described in Japanese Patent Publication No. 36(1961)-9,168; the method involving melting, dispersing and cooling procedures as described in British Patent Nos. 952,807 and 965,074; and the spray drying method as described in U.S. Pat. No. 3,111,407 and British Patent No. 930,422.

Among these encapsulating method, the interfacial polymerization method comprising the following process is preferably employed for the preparation of the toner material of the invention.

In the first place, the following two substances are selected:

Substance (A) which as such is a hydrophobic liquid or a substance soluble, miscible or well dispersable in a hydrophobic liquid; and

Substance (B) which as such is a hydrophilic liquid or a substance soluble, miscible or well dispersable in a hydrophilic liquid, in which Substance (A) can react with Substance (B) to produce polyurethane, polyurea or polythiourethane insoluble in either the hydrophobic liquid or the hydrophilic liquid.

In the second place, very small droplets of a hydrophobic liquid including Substance (A) and the core material containing a colorant and having an average diameter in the range from about 0.5 to about 1,000 microns are dispersed in a hydrophilic liquid such as water containing Substance (B).

A catalyst can be incorporated in either or both of the hydrophobic liquid and the hydrophilic liquid.

The Substance (A) is caused to react with Substance (B) to undergo interfacial polymerization in the dispersion by an appropriate procedure, for instance, by heating the dispersion. Thus, the shells of polyurethane, polyurea or polythiourethane are formed around the hydrophobic droplets including the core material and the colorant, and accordingly the encapsulation of the core material and the colorant with the shell is accomplished to produce encapsulated toner particles in the aqueous liquid.

Examples of Substance (A) preferably employed for the preparation of the shell in the invention include compounds carrying isocyanate or thioisocyanate groups described below:

(1) Diisocyanate

m-phenylenediisocyanate, p-phenylenediisocyanate, 2,6-tolylendiisocyanate, 2,4-tolylendiisocyanate, naphthalene-1,4-diisocyanate, diphenylmethane-4,4'-diisocyanate, 3,3'-dimethoxy-4,4'-biphenyldiisocyanate, 3,3'-dimethyldiphenylmethane-4,4'-diisocyanate, xylylene-1,4-diisocyanate, xylylene-1,3-diisocyanate, 4,4'-diphenylpropanediisocyanate, trimethylenediisocya-

nate, hexamethylenediisocyanate, propylene-1,2-diisocyanate, butylene-1,2-diisocyanate, ethylidynediisocyanate, cyclohexylene-1,2-diisocyanate, cyclohexylene-1,4-diisocyanate, p-phenylenediisocyanate, triphenylmethanediisocyanate;

(2) Triisocyanate

4,4',4"-triphenylmethanetriisocyanate, polymethylenepolyphenyltriisocyanate, toluene-2,4,6-triisocyanate;

(3) Tetraisocyanate

4,4'-dimethyldiphenylmethane-2,2',5,5'-tetraisocyanate;

(4) Polyisocyanate prepolymer

an addition product of hexamethylene diisocyanate and hexanetriol, an addition product of 2,4-tolylendiisocyanate and catechol, an addition product of 2,4-tolylendiisocyanate and hexanetriol, an addition product of 2,4-tolylendiisocyanate and trimethylolpropane, an addition product of xylylenediisocyanate and trimethylolpropane; and

(5) Diisothiocyanate

tetramethylenediisothiocyanate, hexamethylenediisothiocyanate, p-phenylenediisothiocyanate, xylylene-1,4-diisothiocyanate, ethylidynediisothiocyanate.

Examples of the Substance (B) preferably employed for the preparation of the shell in the invention include compounds described below:

(1) Water;

(2) Polyol and polythiol;

ethylene glycol, 1,4-butanediol, catechol, resorcinol, hydroquinone, 1,2-dihydroxy-4-methylbenzene, 1,3-dihydroxy-5-methylbenzene, 3,4-dihydroxy-1-methylbenzene, 3,5-dihydroxy-1-methylbenzene, 2,4-dihydroxy-1-ethylbenzene, 1,3-naphthalenediol, 1,5-naphthalenediol, 2,3-naphthalenediol, 2,7-naphthalenediol, o,o'-biphenol, p,p'-biphenol, 1,1'-bi-2-naphthol, bisphenol A, 2,2'-bis(4-hydroxyphenyl)butane, 2,2'-bis(4-hydroxyphenyl)isopentane, 1,1'-bis(4-hydroxyphenyl)cyclopentane, 1,1'-bis(4-hydroxyphenyl)cyclohexane, 2,2'-bis(4-hydroxy-3-methylphenyl)-propane, bis(2-hydroxyphenyl)-methane, xylylenediol, ethyleneglycol, 1,3-propylene glycol, 1,4-butylene glycol, 1,5-pentanediol, 1,6-heptanediol, 1,7-heptanediol, 1,8-octanediol, trimethylolpropane, hexanetriol, pentaerythritol, glycerol, sorbitol;

(3) Polyamine

ethylenediamine, tetramethylenediamine, pentamethylenediamine, hexamethylenediamine, p-phenylenediamine, m-phenylenediamine, 2-hydroxytrimethylenediamine, diethylenetriamine, triethylenetetraamine, diethylaminopropylamine, tetraethylenepentaamine, an addition product of an epoxy compound and an amine compound; and

(4) Piperazine

piperazine, 2-methylpiperazine, 2,5-dimethylpiperazine.

In the preparation of the dispersion of the very small hydrophobic droplets containing Substance (A) and the core material, the hydrophobic liquid to be dispersed preferably contains a low-boiling solvent or a polar solvent. These solvents serve for accelerating formation of the shell which is a reaction product between the Substance (A) and the Substance (B). Examples of these solvents include methyl alcohol, ethyl alcohol, diethyl ether, tetrahydrofuran, dioxane, methyl acetate, ethyl acetate, acetone, methyl ethyl ketone, methyl isobutyl ketone, cyclohexanone, n-pentane, n-hexane, benzene, petroleum ether, chloroform, carbon tetrachloride,

methylene chloride, ethylene chloride, carbon disulfide and dimethylformamide.

The encapsulated toner material whose shell is composed substantially of a double layer comprising, for instance, a polyurethane, polyurea and/or polythiourethane layer and a polyamide layer can be produced as follows:

In a hydrophobic liquid comprising core materials such as a colorant, a pressure fixable adhesive material (binder), and, if desired, magnetizable particles, are dissolved an acid chloride and a polyisocyanate. This solution is then dispersed in an aqueous medium comprising a polyamine or piperazine and a dispersing agent to produce fine droplets of the core material having an average diameter in the range from about 0.5 to about 1,000 microns in the aqueous medium.

The dispersion produced as above is then neutralized or made weak-alkaline by addition of an alkaline substance, resulting in the formation of a polyamide resin shell (the polyamide substantially is a reaction product of the acid chloride with the polyamine) around the hydrophobic droplet. The dispersion was subsequently heated to a temperature between 40° and 90° C., resulting in the formation of a polyurea resin shell (the polyurea substantially is a reaction product of the polyisocyanate and the polyamine) on the inner surface of the polyamide resin shell. Thus, a double layer shell in which the outer layer is composed substantially of polyamide and the inner layer is composed substantially of polyurea is produced around the hydrophobic core material droplet to give an encapsulated particle.

If a polyol is further added to the hydrophobic liquid in the above, there is produced around the hydrophobic core material droplet a double layer shell in which the outer layer is composed substantially of polyamide and the inner layer is composed substantially of polyurethane (a reaction product of polyisocyanate with polyol).

Alternatively, if the polyisocyanate is replaced with a polyisothiocyanate and a polyol is added to the hydrophobic liquid, there is produced around the hydrophobic core material droplet a double layer shell in which the outer layer is composed substantially of polyamide and the inner layer is composed substantially of polythiourethane (a reaction product of polyisothiocyanate with polyol).

In the latter two procedures, the inner layer composed of a mixture of polyurethane and polyurea or a mixture of polythiourethane and polyurea can be produced, if the polyamine is introduced into the reaction system in an amount exceeding the amount required to react the introduced acid chloride.

The shell of the so produced particle is, as described above, a double layer shell. However, the term "double layer shell" is not intended to mean only a shell in which the two layers are completely separated by a simple interface, but include a shell in which one side, particularly the outer side, of the shell is composed mainly of polyamide, and, another side, particularly the inner side, of the shell is composed mainly of another polymer or other polymers such as polyurethane, polyurea, polythiourethane or a mixture of two or three of these polymers.

Examples of acid chlorides include adipoyl chloride, sebacyl chloride, phthaloyl chloride, isophthaloyl chloride, terephthaloyl chloride, fumaloyl chloride, 1,4-cyclohexanedicarbonyl chloride, 4,4'-biphenyl-dicarbonyl chloride, 4,4'-sulfonyldibenzoyl chloride,

phosgene, polyesters containing acid chloride groups, and polyamides containing acid chloride groups.

The acid chloride can be replaced with a dicarboxylic acid or its acid anhydride. Examples of the dicarboxylic acids include adipic acid, sebacic acid, phthalic acid, terephthalic acid, fumaric acid, 1,4-cyclohexanedicarboxylic acid and 4,4'-biphenyldicarboxylic acid. Examples of the acid anhydrides include phthalic anhydride.

As for the other aspects of the interfacial polymerization method and the other processes for the preparation of micro-capsules containing an oily liquid, there are given descriptions in U.S. Pat. No. 2,726,804, which is introduced hereinto as the reference.

The core material of the invention contains a colorant for producing a visible image from the latent image. The colorant generally is a dye or a pigment, but a certain agent providing no directly visible image such as a fluorescent substance can be employed as the colorant, if desired.

The colorant is generally selected from a variety of the dye, pigment and the like employed generally in the conventional electrostatographic copying and duplicating process. Generally the colorant is a black toner or a chromatic toner. Examples of the black toners include carbon black. Examples of the chromatic toners include blue colorants such as copper phthalocyanine and a sulfonamide derivative dye; yellow colorants such as a benzidine derivative colorant, that is generally called Diazo Yellow; and red colorants such as Rhodamine B Lake that is a double salt of xanthin dye with phosphorus wolframate and molybdate, Carmine 6B belonging to Azo pigment, and a quinacridone derivative.

The core material of the invention further contains a binder for keeping the colorant within the core and assisting the fixing of the colorant onto the surface of a support medium such as paper. The binder is generally selected from high-boiling liquids conventionally employed or proposed for employment for finely dispersing an oil-soluble photographic additive within an aqueous medium to incorporate the additive into a silver halide color photosensitive material, and selected from polymers proposed for employment as the binders for the pressure fixable encapsulated toner materials.

Examples of the high-boiling liquids include the following compounds having the boiling point of higher than 180° C.:

(1) Phthalic esters

dibutyl phthalate, dihexyl phthalate, diheptyl phthalate, dioctyl phthalate, dinonyl phthalate, dodecyl phthalate, butyl phthalyl butyl glycolate, dibutyl monofluorophthalate;

(2) Phosphoric acid esters

tricresyl phosphate, trixylenyl phosphate, tris(isopropylphenyl) phosphate, tributyl phosphate, trihexyl phosphate, trioctyl phosphate, trinonyl phosphate, tridecyl phosphate, trioleyl phosphate, tris(butoxyethyl) phosphate, tris(chloroethyl) phosphate, tris(dichloropropyl) phosphate;

(3) Citric acid esters

O-acetyl triethyl citrate, O-acetyl tributyl citrate, O-acetyl trihexyl citrate, O-acetyl trioctyl citrate, O-acetyl trinonyl citrate, O-acetyl tridecyl citrate, triethyl citrate, tributyl citrate, trihexyl citrate, trioctyl citrate, trinonyl citrate, tridecyl citrate;

(4) Benzoic acid esters

butyl benzoate, hexyl benzoate, heptyl benzoate, octyl benzoate, nonyl benzoate, decyl benzoate, dodecyl benzoate, tridecyl benzoate, tetradecyl benzoate,

hexadecyl benzoate, octadecyl benzoate, oleyl benzoate, pentyl o-methylbenzoate, decyl p-methylbenzoate, octyl o-chlorobenzoate, lauryl p-chlorobenzoate, propyl 2,4-dichlorobenzoate, octyl 2,4-dichlorobenzoate, stearyl 2,4-dichlorobenzoate, oleyl 2,4-dichlorobenzoate, octyl p-methoxybenzoate;

(5) Aliphatic acid esters

hexadecyl myristate, dibutoxyethyl succinate, dioctyl adipate, dioctyl azelate, decamethylene-1,10-diol diacetate, triacetin, tributin, benzyl caprate, pentaerythritol tetracaprate, isosorbitol dicaprilate;

(6) Alkylnaphthalenes

methylnaphthalene, dimethylnaphthalene, trimethylnaphthalene, tetramethylnaphthalene, ethynaphthalene, diethylnaphthalene, triethylnaphthalene, monoiso-propylnaphthalene, diisopropylnaphthalene, tetraiso-propylnaphthalene, monomethylethynaphthalene, isoctylnaphthalene;

(7) Dialkylphenyl ethers

di-o-methylphenyl ether, di-m-methyldiphenyl ether, 20 di-p-methylphenyl ether;

(8) Amides of fatty acids and aromatic sulfonic acid N,N-dimethyllauroamide, N,N-diethylcaprylamine, N-butylenzenesulfonamide;

(9) Trimellitic acid esters

triocetyl trimellitate;

(10) Diarylalkanes

diarylmethanes, e.g., dimethylphenylphenylmethane, diarylethanes, e.g., 1-methylphenol-1-phenylethane, 1-dimethylphenyl-1-phenylethane, 1-ethylphenyl-1-30 phenylethane.

The above-listed high-boiling liquids and examples of other high-boiling liquids employable in the invention are described in detail in the following publications:

Japanese Patent Publications No. 46(1971)-23,233 and 35 No. 49(1974)-29,461; Japanese Patent Provisional Publication Nos. 47(1972)-1,031, 50(1975)-62,632, 50(1975)-82,078, 51(1976)-26,035, 51(1976)-26,036, 51(1976)-26,037, 51(1976)-27,921, and 51(1976)-27,922; U.S. Pat. Nos. 2,322,027, 2,353,262, 2,533,514, 40 2,835,579, 2,852,383, 3,287,134, 3,554,755, 3,676,137, 3,676,142, 3,700,454, 3,748,141, 3,837,863, and 3,936,303; British Patent Nos. 958,441, 1,222,753, 1,346,364, and 1,389,674; and West Germany Offenlegungsschrift No. 2,538,889.

For the purpose of the invention, the high-boiling liquid is preferably selected from the phthalic acid esters, phosphoric acid esters and alkylnaphthalenes.

Examples of the polymers include the following polymers:

polyolefins, olefin copolymers, polystyrene, styrenebutadiene copolymer, epoxy resins, polyesters, natural and synthetic rubbers, polyvinylpirolidone, polyamides, cumarone-indene copolymer, methyl vinyl ether-maleic anhydride copolymer, maleic acid-modified phenol resin, phenol-modified terpene resin, silicone resins, epoxymodified phenol resin, amino resins, polyurethane elastomers, polyurea elastomers, homopolymers and copolymers of acrylic acid ester, homopolymers and copolymers of methacrylic acid ester, acrylic acid-long chain alkyl methacrylate copolymer oligomer, poly(vinyl acetate), and poly(vinyl chloride).

The above-listed polymers and examples of other polymers employable in the invention are described in detail in the following publications:

Japanese Patent Publication Nos. 48(1973)-30,499, 49(1974)-1,588 and 54(1979) -8,104; Japanese Patent Provisional Publication Nos. 48(1973)-75,032,

48(1973)-78,931, 49(1974)-17,739, 51(1976)-132,838, 52(1977)-98,531, 52(1977)-108,134, 52(1977)-119,937, 53(1978)-1,028, 53(1978)-36,243, 53(1978)-118,049, 55(1980)-89,854 and 55(1980)-166,655; and U.S. Pat. Nos. 3,788,994 and 3,893,933.

The core material can further contain other agents such as a releasing agent and magnetizable particles.

The releasing agent serves for keeping the ruptured shell and the released core material from adhering to the surface of the pressing roller. The releasing agent can be chosen from those proposed for employment in the previously reported encapsulated toners. Examples of the releasing agents include a fluorine-containing resin described in Japanese Patent Provisional Publication Nos. 55(1980)-142,360 and 55(1980)-142,362.

The magnetizable particles are included in the core material where a magnetizable toner material for the one component developing process is desired. As for the magnetizable particles, there are descriptions, for instance, in Japanese Patent Provisional Publication Nos. 53(1978)-118,053, 53(1978)-1,028 and 55(1980)-166,655. Examples of materials of the magnetizable particles preferably employed in the invention include metals such as cobalt, iron and nickel; metal alloys or metal compositions comprising aluminum, cobalt, copper, iron, lead, magnesium, nickel, tin, zinc, gold, silver, antimony, beryllium, bismuth, cadmium, calcium manganese, titanium, tungsten, vanadium and/or zirconium; metallic compounds including metal oxides such as aluminium oxide, ferric oxide, cupric oxide, nickel oxide, zinc oxide, zirconium oxide, titanium oxide and magnesium oxide; refractory metal nitrides such as chromium nitride; metal carbides such as tungsten carbide and silicon carbide; ferro-magnetic ferrite; and their mixtures.

As mentioned hereinbefore, a process for the preparation of the encapsulated toner particles includes a stage for dispersing or emulsifying very small droplets of the hydrophobic liquid containing Substance (A) and the core material in the aqueous medium. For the preparation of the homogeneous dispersion (or, emulsion) of the very small droplets of the hydrophobic liquid, it is preferred to incorporate into the reaction liquid a hydrophilic protective colloid and/or an emulsifying surface active agent which assist the production of the homogeneous dispersion (or, emulsion) of the hydrophobic droplets and prevention of agglomeration of the so-produced hydrophobic droplets. The hydrophilic protective colloid and the surface active agent can be employed alone or in combination.

Examples of the preferred hydrophilic protective colloids include proteins such as gelatin, graft polymers of gelatin and other polymers, albumin, and casein; cellulose derivatives such as hydroxyethylcellulose, carboxymethylcellulose, and cellulose sulfuric acid ester; saccharide derivatives such as sodium alginate and starch derivatives; and a variety of synthetic hydrophilic homopolymers and copolymers such as polyvinyl alcohol, partially acetalized polyvinyl alcohol, poly-N-vinyl pyrrolidone, polyacrylic acid, polyacrylic amide, polyvinylimidazole and polyvinylpyrazole.

In the above-listed examples, the gelatin can be a lime-treated gelatin, an acid-treated gelatin, a hydrolyzed gelatin, and an enzymically decomposed gelatin.

The graft polymers of gelatin and other polymers can be gelatins carrying graft chains consisting of homopolymers or copolymers of vinyl monomers such as acrylic acid, methacrylic acid, their derivatives, e.g., esters and

amides, acrylonitrile, and styrene. Examples of the gelatin graft polymers are those miscible with gelatin such as the gelatins carrying the graft chains consisting of polymers of acrylic acid, methacrylic acid, acrylamide, methacrylamide and hydroxyalkyl methacrylate.

Details of these preferred gelatin graft polymers are described in U.S. Pat. Nos. 2,763,625, 2,831,767, and 2,956,884.

Representative examples of the synthetic hydrophilic polymers are described, for instance, in West German Offenlegungsschrift No. 2,312,708, U.S. Pat. Nos. 3,620,751 and 3,879,205, and Japanese Patent Publication No. 43(1968)-7,561.

The surface active agents for dispersing or emulsifying the hydrophobic liquid in the hydrophilic liquid medium can be incorporated into either or both of the hydrophobic liquid and the hydrophilic liquid medium.

Examples of the surface active agents include non-ionic surface active agents, for instance, saponin (steroid type), alkylene oxide derivatives such as polyethylene glycol, polyethylene glycol/polypropylene glycol condensation product, alkyl- or alkylarylether of polyethylene glycol, polyethylene glycol esters, polyethylene glycol sorbitol ester, alkylamine or amide of polyalkylene glycol, polyethylene oxide adduct of silicone polymer, glycidol derivatives such as polyglyceride alkenylsuccinate and alkylphenol polyglyceride, fatty acid esters of polyhydric alcohols, alkylesters of saccharide, urethanes and ethers; and anionic surface active agents having acidic groups such as carboxy, sulfo, phospho, sulfate ester and phosphate ester groups, for instance, triterpenoide-type saponin, alkylcarboxylic acid salts, alkylsulfonic acid salts, alkylbenzenesulfonic acid salt, alkylphthalenesulfonic salts, alkylsulfate esters, alkylphosphate esters, N-acyl-N-alkyl-taurines, sulfosuccinic acid esters, sulfoalkyl-polyoxyethylene alkylphosphate esters.

Particularly preferred surface active agents are anionic surface active agents belonging to the sulfonic acid type and the sulfate ester type, namely, compounds having in the molecular structure both of hydrophobic groups containing 8-30 carbon atoms and hydrophilic groups of  $-\text{SO}_3\text{M}$  or  $-\text{OSO}_3\text{M}$  (in which M is Na or K). These preferred anionic surface active agents belonging to the above-mentioned types are described in detail in "Surface Active Agents" (A. W. Perry; Interscience Publication Inc., New York).

Representative examples of the preferred anionic surface active agents are as follows: sodium dodecylsulfate, sodium tetradecylsulfate, Turkey red oil, sodium dodecylcarboxyamidoethylsulfate, sodium dodecylsulfonate, sodium tetradecylsulfonate, sodium polyoxyethylene-octylphenyl-ethersulfonate, sodium salt of sulfosuccinic acid diocylester, sodium dodecylbenzenesulfonate, sodium tetradecylamidophenylsulfonate, and sodium tri-isopropylnaphthalenesulfonate.

Dispersing or emulsifying the reaction liquid can be carried out by means of a known homogenizer such as one belonging to the stirring type, the high pressure injecting type, the ultrasonic vibrating type and the kneader type. Particularly preferred homogenizers are a colloid mill, a conventional homogenizer, and electromagnetic distortion inducing ultrasonic homogenizer.

The encapsulated toner is then produced, for instance, by heating the emulsified reaction liquid in the presence of an appropriate catalyst, as described hereinbefore, so as to form shells around the core material

droplets. Subsequently, the encapsulated toner is separated from the aqueous reaction medium and dried to obtain a dry encapsulated toner. The encapsulated toner is preferably washed with water after the separation from the aqueous reaction medium and prior to the drying procedure. The drying procedure can be carried out by a known process such as the spray-drying process or the freeze-drying process. The spray-drying process is preferred.

The so-produced dry encapsulated toner can be admixed with an insulating material and/or a charge controller such as a metal-containing dye or Nigrosine dye.

The dry encapsulated toner can be admixed with a flow lubricant such as hydrophobic silica powder so that the flow lubricant can be dispersed over the surface of the encapsulated toner. The encapsulated toner having the flow lubricant such as hydrophobic silica powder over the toner surface shows particularly improved powder quality and property, and accordingly is very advantageous in the practical use.

The encapsulated toner obtained as above can be introduced into the electrostatographic copying and duplicating machine to develop an electrostatographically produced latent image so as to produce a visible toner image on the surface of the photoconductive material. The visible image is then fixed onto a support medium such as paper by means of an appropriate pressure fixing apparatus. There is no limitation on the pressure fixing apparatus for fixing the encapsulated toner of the invention, and any known apparatus can be applied to the fixing of the encapsulated toner of the invention. Examples of the pressure fixing apparatuses include those illustrated in Japanese Patent Publication Nos. 44(1969)-9,880, 44(1969)-12,797, 46(1971)-15,876; and Japanese Patent Provisional Publication Nos. 49(1974)-6 2,143, 49(1974)-77,641, 50(1975)-51,333, 51(1976)-31,235, 51(1976)-40,351, 52(1977)-15,335, 52(1977)-102,743, 54(1979)-28,636, 54(1979)-32,326, 54(1979)-41,444, and 54(1979)-48,251.

The electrostatographic toner material comprising the encapsulated toner particles of the invention has improved powder characteristics, and is resistant to the mechanical shock and abrasion in the developing apparatus of the electrostatographic copying and duplicating machine. Further, the electrostatographic toner material of the invention is easily rupturable in the pressure fixing apparatus to produce a visible toner image well fixed onto the support medium such as paper. Furthermore, the toner material of the invention hardly undergoes offsetting to a pressing roller and hardly undergoes the so-called filming on the surfaces of the carrier particles, the developing sleeves and the photoconductive material.

In the employment for the two component developing process, the toner material of the invention can be appropriately charged to carry an electric charge in the range of 10-20  $\mu\text{c/g}$  (plus or minus) in combination with an adequate carrier or with an adequate charge controller, so as to provide a visible image fixed on a support medium with high quality such as high resolution and high sharpness with substantially no fog. The development characteristics and the pressure fixability of the toner material of the invention are kept at an excellent level even after copying and duplicating procedure is repeated to a certain extent.

Even in the employment for the one component developing process, the toner material of the invention is well qualified in the developing characteristics, the

pressure fixing characteristics and the resistance to the offsetting. Moreover, no filming is produced on the surfaces of the development sleeve and the photosensitive material.

Other features of the electrostatographic copying and duplicating process employing an encapsulated toner material are described in U.S. Pat. No. 3,788,994, which is introduced hereinto as the reference.

The present invention will be illustrated by the following examples which are by no means intended to 10 introduce any restriction into the invention.

#### EXAMPLE 1

Into a dispersion of 3 g. of carbon black in 27 g. of dibutyl phthalate was introduced 10 g. of a mixture of 15 acetone and methylene chloride (1:3, volume ratio), and the mixture was then admixed to become homogeneous.—Primary liquid.

Subsequently, 4 g. of an adduct of hexamethylene diisocyanate with hexanetriol (3:1 molar ratio adduct) 20 and 0.05 g. of dibutyltin laurate (catalyst) were added to the primary liquid at room temperature.—Secondary liquid.

Independently, 3 g. of gum arabic was dissolved in 57 g. of water at 20° C., and into this solution under vigorous stirring was poured little by little the secondary liquid. Thus, there was obtained an oil-in-water emulsion containing oily droplets having average diameter of 5-15μ. The procedure for the preparation of the emulsion was carried out under cooling the reaction 30 vessel for keeping the temperature of the emulsion below 20° C.

To the emulsion was further added under stirring 100 g. of water heated to 40° C. After completion of the addition of water, the emulsion was gradually heated to 35 90° C. over 30 min. The emulsion was kept under stirring at the temperature for 20 min. so as to complete the encapsulating reaction.

The dispersion containing the encapsulated oily particles was subjected to centrifugal separation at 5,000 40 r.p.m. to separate the encapsulated particles from the aqueous gum arabic solution. To the so separated particles were added 100 cc. of water and 10 cc. of a mixture of isopropyl alcohol and water (1:1) containing 2% by weight of di-2-ethylhexyl sodium sulfosuccinate, and the so produced dispersion was dried in a spray-drying apparatus to obtain a powder encapsulated toner material.

The encapsulated toner material obtained above was composed of a core containing the carbon black and dibutyl phthalate and a shell made substantially of a reaction product of the adduct of hexamethylene diisocyanate with hexanetriol and water. Microscopic observation of the encapsulated toner indicated that most of the toner particles were present independently and that no bulky agglomerated particles were formed.

The evaluation of the encapsulated toner was carried out as follows.

Five parts by weight of the toner were admixed with 95 parts by weight of powdery iron carrier in a shaking 60 apparatus to prepare a developing agent. It was confirmed through microscopic observation that the developing agent contained no ruptured toner particles.

A conventional electrostatographic copying and duplicating process was carried out using the above developing agent. The visible toner image produced on a latent image was then converted onto a paper. The paper carrying the toner image was treated under a

pressing roller at a pressure of 350 kg/cm<sup>2</sup>. There was obtained a toner image with high sharpness and well fixed onto the paper. Further, the off-setting of the toner was at a very low level.

#### EXAMPLE 2

In a dispersion of 1 g. of carbon black in 13 cc. of tricresyl phosphate was dissolved 1 g. of an adduct of tolylene diisocyanate with hexanetriol (3:1 molar ratio adduct) to prepare a primary liquid.

Independently, 7 g. of polyvinyl alcohol was dissolved in 100 cc. of water to prepare a secondary liquid.

The primary liquid was dropped into the secondary liquid under stirring to disperse very small droplets of the primary oily liquid in the secondary liquid. The mixture was further emulsified under stirring at room temperature for approximately 2 hours followed by stirring at 80° C. for approximately 1 hour. While the stirring was carried out, the diisocyanate adduct reacted with water to produce insoluble shells enclosing the oily droplets to yield encapsulated toner particles.

The dispersion containing the encapsulated oily particles was then treated in the same manner as described in Example 1 except for employing diisohexyl sodium sulfosuccinate to obtain a powdery encapsulated toner material.

The encapsulated toner material obtained above was composed of a core containing the carbon black and tricresyl phosphate and a shell made substantially of a reaction product of the adduct of tolylene diisocyanate with hexanetriol and water. Microscopic observation of the encapsulated toner indicated that most of the toner particles were present independently and that no bulky agglomerated particles were formed.

The evaluation of the encapsulated toner as the developing agent was carried out in the same manner as described in Example 1. It was confirmed that substantially no ruptured toner particles were seen upon mixing with the powdery iron carrier. Also confirmed was that a toner image with sharpness was well fixed onto a paper. The off-setting of the toner was kept at a very low level.

We claim:

1. An electrostatographic toner material for a pressure fixing process comprising powdery encapsulated toner particles having an average particle size in the range from about 0.5 to about 1,000 microns, in which the toner particle comprises a pressure fixable adhesive core material containing a colorant and a pressure rupturable shell enclosing the core material, the outer surface of the shell being provided with a surface active agent having the following hydrophobic group:



in which R<sup>1</sup> and R<sup>2</sup> are the same or different, and each is an aliphatic hydrocarbon group of 2-20 carbon atoms or an aromatic hydrocarbon group of 6-20 carbon atoms.

2. The electrostatographic toner material as claimed in claim 1, in which each of R<sup>1</sup> and R<sup>2</sup> is an aliphatic hydrocarbon group of 4-12 carbon atoms or an aromatic hydrocarbon group of 6-12 carbon atoms.

3. The electrostatographic toner material as claimed in claim 2, in which each of R<sup>1</sup> and R<sup>2</sup> is an aliphatic hydrocarbon group of 6-10 carbon atoms.

4. The electrostatographic toner material as claimed in claim 1, in which the surface active agent contains at least one hydrophilic group selected from the group consisting of sulfonate, carboxylate, phosphate, amine, quaternary ammonium salt and pyridinium salt.

5. The electrostatographic toner material as claimed in claim 4, in which the surface active agent contains at least one hydrophilic sulfonate group.

6. The electrostatographic toner material as claimed in claim 1, in which the shell is made of a polymer selected from the group consisting of polyurethane, polyurea and polythiourethane.

7. The electrostatographic toner material as claimed in claim 6, in which the shell is made substantially of a polycondensation product of polyisocyanate, polyol and water.

8. The electrostatographic toner material as claimed in claim 6, in which the shell is made substantially of a polycondensation product of polyisocyanate, polyol and polyamine.

9. The electrostatographic toner material as claimed in claim 1, in which the shell is composed substantially of a double layer comprising a polyurethane, polyurea and/or polythiourethane layer and a polyamide layer.

10. The electrostatographic toner material as claimed in claim 1, in which the pressure fixable adhesive core material is a liquid medium boiling at a temperature of higher than 180° C.

11. The electrostatographic toner material as claimed in claim 1, in which a flow lubricant is provided onto the surface of the shell.

\* \* \* \* \*

20

25

30

35

40

45

50

55

60

65